

June 23, 1931.

W. F. GRAHAM

1,811,388

TROLLEY SHOE

Filed June 10, 1930



FIG. 1



FIG. 2



FIG. 3



FIG. 4

Witness:

*W. P. Sparks*

By

WALTER F. GRAHAM Inventor

*Graham* Attorney

Patented June 23, 1931

1,811,388

# UNITED STATES PATENT OFFICE

WALTER F. GRAHAM, OF RICHLAND, OHIO, ASSIGNOR TO THE OHIO BRASS COMPANY, OF MANSFIELD, OHIO, A CORPORATION OF NEW JERSEY

## TROLLEY SHOE

Application filed June 10, 1930. Serial No. 460,204.

My invention relates to a trolley shoe or current collector which slides along the trolley wire.

The object of my invention is to provide a shoe of ferrous metal which will possess hardened areas as compared with other areas to increase the life of the shoe and remove probability of the shoes breaking or cracking as is the case where the entire shoe is hardened.

Shoes of the character shown and described herein are ordinarily made from low carbon steel, case hardened all over. This case hardening process if the one usually employed, 15 namely that of packing the steel forging in a carbonaceous material such as charcoal, pulverized carbon, etc. and holding the article for a pre-determined period of time at a temperature in the neighborhood of 1650° F., thereby obtaining a penetration of the 20 carbon into the steel which is commonly referred to as a carburization or cementation of the steel, it will be found that the entire surface has been penetrated to approximately 25 by  $\frac{1}{16}$ " to  $\frac{1}{8}$ " with increased carbon and such pieces are hardened by quenching in a suitable medium as oil or water from above the critical point.

When shoes are prepared as outlined above, 30 we find that not only is the wearing surface in the groove highly hardened, but the lips or thinner portions forming the groove are extremely brittle and such shoes are not entirely suitable for the purpose intended due 35 to certain portions being hardened which could better be left unhardened.

Also, we find that if it is attempted to draw the hardness of those portions which it is 40 undesirable to have hardened as by subjecting the shoe to a temperature of from 500° to 600° F., that such temperature would be sufficient to reduce the hardness not only in the flanges, but also in the bottom of the groove or wearing portion.

45 After analyzing the difficulties met with in standard shoes as described above and considerable experimental work I found I was able to produce a shoe which had only those portions desired highly hardened while 50 other portions were relatively soft.

In producing a shoe of this character my process broadly is to coat those surfaces which I do not wish to be hardened with a material which will prevent the carbon passing through and entering the steel. 55

In the accompanying drawing:—

Fig. 1 is a side view of one form of trolley shoe.

Fig. 2 is an end view of Fig. 1.

Fig. 3 is an opposite end view of Fig. 1. 60

Fig. 4 is a transverse sectional view on the line 4—4 of Fig. 1 and shows the relative hardness of different portions of the shoe on the line 4—4 of Fig. 1. 65

I might term my shoe a selectively case hardened shoe and such shoe is produced by preventing the penetration of the carbon in the sections or areas of the device in which the high carbon material would be either unnecessary or injurious after the hardening process. 70

While there may be various methods of producing selective hardening the process which I prefer to use is that of first cleaning the forging to remove all scale; then to copper plate the forging over its entire surface with a heavy coat of copper from a cyanide copper solution; then I remove the copper by grinding or wire brushing from such portions which I desire the carbon to penetrate 80 into during the carburizing operation; this same result may be secured by painting or japanning those portions which are to be penetrated by the carbon, before copper plating and then removing the paint or japan after plating, thus leaving the portions to be hardened, free of copper; to then place the prepared shoe in a carbonaceous compound which will not attack the copper plate as for example hydro-carbonate of boneblack, and 90 at a temperature of approximately 1650° F. for a sufficient length of time to obtain a penetration of the copper of approximately  $\frac{3}{32}$ " in the mild steel; then machine such portions of the forging as necessary. The machining 95 operation, however, may be carried out before the carburizing process; then the carburized and machined shoe is hardened by giving it a double quench, that is, by first heating the shoe to approximately 1550° to 100

1600° F., and then quenching in either water or oil, preferably the latter and this gives the shoe a refined low carbon core. The high carbon portion is then hardened and refined by heating to about 1425° F. and quenching in water. The shoe is then subjected to a low drawing heat at a temperature under 375° F. which will remove hardening strains, but will be sufficiently low to prevent the change of the martensitic structure to the softer troostitic structure.

The shoe produced as above described will be of mild steel, that is, with carbon not over .25% with a hard wearing surface or surfaces which come in contact with the trolley wire and soft, ductile portions which are liable to be subjected to shocks or blows.

The locations of the high carbon material can best be illustrated in the figures referred to. In Fig. 4 the high carbon portions are represented by the numerals 1 and 2 and the soft core structure by the numeral 3 and the flanges as 4. The longitudinal extent of the hardened portion which may be indicated in Fig. 1 by the dotted line 5 and that of the hardened portion 2 by the dotted line 6.

When the shoe is new the hardened portion which engages the trolley wire will of course after a period of time become worn through and the softer portion 3 will then contact with the trolley wire. The shoe is so constructed that the entire central portion may be worn through before it is necessary to remove the shoe and therefore in order to give the user the benefit of the selective hardening the longitudinal central portion of the shoe below the hardened portion 1 is likewise hardened and therefore when the trolley wire has cut through the portions 1 and 3 it again contacts with a hardened portion 2 thereby decreasing the rate of wear.

Shoes have been made of high carbon steel which are, when hardened, of uniform hardness throughout but such shoes are not satisfactory as they check in hardening or they break through shocks and blows when in service, but with a shoe constructed as described herein of low carbon steel such breakages are avoided and at the same time the wearing portions are given increased life.

In order to prevent the penetration of carbon into the steel body or certain desired places it is possible to coat such places with a slip made of clay, that is, a solution of clay and water, silicate of soda, or other suitable liquid. Also in place of using a copper coating, a coating of other non-ferrous metal which will prevent the passage of carbon and withstand the carburizing temperature may be used.

If desired the entire inner surface of the groove may be formed of hardened material which would be merely that of continuing the hardened portion 1 or if desired the shoe 35 may be made of mild steel with the entire

surface hardened leaving a soft mild steel core, but I prefer a shoe having only the portion 1 hardened or the portions 1 and 2, leaving in both cases the upstanding lips 4 unhardened and of mild steel.

If the portion through the bottom of the groove is not too thick, the portions 1, 2 and 3 may be made hard by my process and the lips 4 left soft.

If the material used is a low carbon steel with an alloy content, that is, carbon up to .25% and nickel, chromium, vanadium, etc. of 4% more or less, the characteristics of the shoe will be considerably changed by the alloy content of nickel, etc., that is tougher and harder in the parts 1, 2 and 3 and tougher in the lips 4 as compared with carbon steel described.

Modifications will be apparent to those skilled in the art, but I wish to be limited only by my claims.

I claim:—

1. A trolley shoe comprising a body of ferrous material having a grooved portion with an elongated surface to receive and engage a trolley wire, a portion of the body forming said grooved surface having a higher carbon content than the other portions of the shoe.

2. A trolley shoe comprising a body of ferrous material having a grooved portion with an elongated surface to receive and engage a trolley wire, a portion of the body forming said grooved surface having a higher carbon content than the other portions of the shoe and the said higher carbon content portion being harder than the other portions.

3. A trolley shoe comprising a body of mild steel with an elongated grooved portion having a surface to contact with a trolley wire and the portion of the body forming the said surface having a higher carbon content than the portions of the body adjacent the contact surface.

4. A trolley shoe comprising a body of mild steel and having a grooved portion, a portion of the surface within the groove being engaged by a trolley wire and an exterior surface spaced from the said grooved surface, a portion of the body forming the said internal surface and the external surface having a higher carbon content than the intermediate portion of the shoe.

5. A trolley shoe comprising a body of mild steel and having a grooved portion, a portion of the surface within the groove being engaged by a trolley wire and an exterior surface spaced from the said grooved surface, a portion of the body forming the said internal surface and the external surface having a higher carbon content than the intermediate portion of the shoe, the higher carbon content portions having a higher degree of hardness than the intermediate portion.

6. A trolley shoe of a single piece of fer-

- rous metal having two spaced wearing portions and an intermediate portion, the spaced portions having a higher carbon content than the intermediate portion.
- 5 7. A trolley shoe of a single piece of ferrous metal having a grooved portion to slidably engage a conductor, the grooved portion provided with a surface normally contacting with the conductor and upstanding lips, the 10 lips being of mild steel and the portion forming the contacting surface being hard.
8. A trolley shoe of a single piece of alloy steel having a groove with a surface to engage a trolley conductor, a portion of the 15 shoe having a higher carbon content than the other portion of the shoe forming the balance of the surface and hardened.
9. A trolley shoe having a U shaped grooved portion, the lips of the groove being 20 of mild steel and the other portion of the groove being of higher carbon hardened steel.
10. A trolley shoe of hardened steel having a grooved portion with upstanding side 25 walls of mild steel.
11. The method of forming a trolley shoe comprising forging a body of mild steel to proper shape having an elongated portion of U shaped cross-section, then coating certain 30 portions with a material which will prevent the passage of carbon therethrough, then packing the shoe in a carbonaceous material, then subjecting the shoe and material to a sustained temperature for a predetermined 35 time to obtain a penetration of carbon from the carbonaceous material into the shoe and increase the carbon content at the uncoated portions.
12. The method of forming a trolley shoe 40 comprising forging a body of mild steel to proper shape having an elongated portion of U shaped cross-section, then coating certain portions with a material which will prevent the passage of carbon therethrough, then 45 packing the shoe in a carbonaceous material, then subjecting the shoe and material to a sustained temperature for a predetermined time to obtain a penetration of carbon from the carbonaceous material into the shoe and 50 increase the carbon content at the uncoated portions, then quenching the shoe from an elevated temperature to harden those portions having excess carbon.
- 55 13. The method of forming a trolley shoe comprising forging a body of mild steel to proper shape having an elongated portion of U shaped cross-section, then coating certain 60 portions with a plating of non-ferrous metal which will prevent the passage of carbon therethrough, then packing the shoe in a carbonaceous material, then subjecting the shoe and material to a sustained temperature for a predetermined time to obtain a penetration of carbon from the carbonaceous ma- 65
- terial into the shoe and increase the carbon content at the uncoated portion.
14. The method of forming a trolley shoe comprising forging a body of mild steel to proper shape having an elongated portion of U shaped cross-section, then coating certain 70 portions with a plating of copper which will prevent the passage of carbon therethrough, then packing the shoe in a carbonaceous material, then subjecting the shoe and material 75 to a sustained temperature for a predetermined time to obtain a penetration of carbon from the carbonaceous material into the shoe and increase the carbon content at the uncoated portion.
15. A trolley shoe of mild steel having its 80 wearing portions of hardened steel.
16. A grooved trolley shoe comprising a body of mild steel of a carbon content up to .25% and having a portion subjected to wear through contact with a trolley wire, the said portion having a higher carbon content and of a greater hardness than the adjacent portion.
17. A trolley shoe of alloy steel having a 85 carbon content up to .25% and an alloying material up to 4% and having its wearing portion harder than other portions.
- In testimony whereof I affix my signature.
- WALTER F. GRAHAM.
- 100
- 105
- 110
- 115
- 120
- 125
- 130